# NEW EUROPEAN PATENT SPECIFICATION

(11) **EP 0 679 114 B2**
(45) Date of publication and mention of the opposition decision: **03.11.2004**
(45) Mention of the grant of the patent: 21.07.1999
(21) Application number: 95900015.9
(22) Date of filing: 09.11.1994
(51) Int. Cl.: B22D 11/06

(54) **CASTING STAINLESS STEEL STRIP ON SURFACE WITH SPECIFIED ROUGHNESS**
GIESSEN EINES KONTINUIERLICHEN STAHLBANDES AUF EINE OBERFLÄCHE MIT BESTIMMTER RAUHIGKEIT
COULEE D'UNE BANDE D'ACIER INOXYDABLE SUR UNE SURFACE A RUGOSITE PREDETERMINEE

(30) Priority: 18.11.1993 AU PM253993
(43) Date of publication of application: 02.11.1995
(73) Proprietor: Castrip, LLC, Charlotte, NC 28211 (US)
(72) Inventor: MAHAPATRA, Rama Ballav, Yarrawarrah, NSW 2233 (AU); FREEMAN, John, Kahibah, NSW 2290 (AU); STREZOV, Lazar, Adamstown Heights, NSW 2289 (AU)
(74) Representative: Lerwill, John
(86) International application number: PCT/AU1994/000685
(87) International publication number: WO 1995/013889

(56) References cited:
- EP-A- 0 378 705
- EP-A- 0 481 481
- WO-A-93/08941
- AU-A- 2 992 992
- US-A- 5 082 046
- "Thin strip casting experiments at IRSID and Thyssen Stahl AG", Iron and steelmaker, pp. 27-32, August 1993

## Description

This invention relates to the continuously casting of austenitic stainless steel strip. It has particular but not exclusive application to continuous casting of stainless steel strip in a twin roll caster.

It is known to cast metal strip by continuous casting in a twin roll caster. Molten metal is introduced between a pair of contra-rotated horizontal casting rolls which are cooled so that metal shells solidify on the moving roll surfaces and are brought together at the nip between them to produce a solidified strip product delivered downwardly from the nip between the rolls. The term "nip" is used herein to refer to the general region at which the rolls are closest together. The molten metal may be poured from a ladle into a smaller vessel from which it flows through a metal delivery nozzle located above the nip so as to direct it into the nip between the rolls, so forming a casting pool of molten metal supported on the casting surfaces of the rolls immediately above the nip. This casting pool may be confined between side plates or dams held in sliding engagement with the ends of the rolls.

Twin roll casting has been applied with some success to non-ferrous metals which solidify rapidly on cooling, for example aluminium. Our Australian Patent No 631728 discloses a method and apparatus which enables continuous casting of ferrous strip within 0.5 mm to 5 mm and apparatus of this type has been developed to the stage where it is possible to consistently produce good quality mild steel strip. However there have been particular problems in casting austenitic stainless steel strip because of the marked tendency for such steel to suffer from cracking and repetitive surface depressions appearing as a surface defect generally known as "crocodile skin". We have undertaken extensive experimental work in which we have determined factors which make it possible consistently to cast austenitic stainless steel strip of good surface quality without significant cracking defects.

In the ensuing description it will be necessary to refer to a quantitative measure of the smoothness of casting surfaces. One specific measure used in our experimental work and helpful in defining the scope of the present invention is the standard measure known as the Arithmetic Mean Roughness Value which is generally indicated by the symbol Rₐ. This value is defined as the arithmetical average value of all absolute distances of the roughness profile from the centre line of the profile within the measuring length lₘ. The centre line of the profile is the line about which roughness is measured and is a line parallel to the general direction of the profile within the limits of the roughness-width cut-off such that sums of the areas contained between it and those parts of the profile which lie on either side of it are equal. The Arithmetic Mean Roughness Value may be defined as

### DISCLOSURE OF THE INVENTION

According to the invention there is provided a method as defined in claim 1. The surface of this texture may be produced by the machining of regular ridges in the surface.

Preferably the chromium to nickel ratio is no greater than 1.55.

More specifically the invention provides a method as defined in claim 7.

The casting surfaces of the rolls may have a texture of regular circumferential grooves with a texture depth in the range 10 microns to 60 microns and a groove pitch in the range 100 microns to 200 microns.

In an alternative embodiment, the roll may have a texture of regularly spaced projections, which may take the form of pyramids or cones with pitch spacing in the range 100 to 200 microns and depth in the range 10 to 60 microns.

It is preferred that the carbon, chromium and nickel contents of the steel be in the following ranges:

| | |
|---|---|
| Carbon - | 0.04 - 0.06 % by weight |
| Chromium - | 17.5 - 19.5 % by weight |
| Nickel - | 8.0 - 10.0 % by weight. |

### BRIEF DESCRIPTION OF THE DRAWINGS

In order that the invention may be more fully explained its application to the production of stainless steel strip in a twin roll continuous caster will be explained with reference to the accompanying drawings in which:
Figure 1 is a plan view of a twin roll continuous strip caster which may be operated in accordance with the present invention;
Figure 2 is a side elevation of the strip caster shown in Figure 1;
Figure 3 is a vertical cross-section on the line 3-3 in Figure 1;
Figure 4 is a vertical cross section on the line 4-4 in Figure 1;
Figure 5 is a vertical cross-section on the line 5-5 of Figure 1;
Figure 6 illustrates the textured surface of a casting surface used in a series of trial casts; and
Figures 7 to 9 illustrate the results of the trial casts using steels of varying compositions.

### DETAILED DESCRIPTION OF THE PREFERRED EMBODIMENT

The illustrated caster comprises a main machine frame 11 which stands up from the factory floor 12. Frame 11 supports a casting roll carriage 13 which is horizontally movable between an assembly station 14 and a casting station 15. Carriage 13 carries a pair of parallel casting rolls 16 to which molten metal is supplied during a casting operation from a ladle 17 via a tundish 18 and delivery nozzle 19. Casting rolls 16 are water cooled so that shells solidify on the moving roll surfaces and are brought together at the nip between them to produce a solidified strip product 20 at the roll outlet. This product is fed to a standard coiler 21 and may subsequently be transferred to a second coiler 22. A receptacle 23 is mounted on the machine frame adjacent the casting station and molten metal can be diverted into this receptacle via an overflow spout 24 on the tundish or by withdrawal of an emergency plug 25 at one side of the tundish if there is a severe malformation of product or other severe malfunction during a casting operation.

Roll carriage 13 comprises a carriage frame 31 mounted by wheels 32 on rails 33 extending along part of the main machine frame 11 whereby roll carriage 13 as a whole is mounted for movement along the rails 33. Carriage frame 31 carries a pair of roll cradles 34 in which the rolls 16 are rotatably mounted. Roll cradles 34 are mounted on the carriage frame 31 by interengaging complementary slide members 35, 36 to allow the cradles to be moved on the carriage under the influence of hydraulic cylinder units 37, 38 to adjust the nip between the casting rolls 16. The carriage is movable as a whole along the rails 33 by actuation of a double acting hydraulic piston and cylinder unit 39, connected between a drive bracket 40 on the roll carriage and the main machine frame so as to be actuable to move the roll carriage between the assembly station 14 and casting station 15 and vice versa.

Casting rolls 16 are contra rotated through drive shafts 41 from an electric motor and transmission mounted on carriage frame 31. Rolls 16 have copper peripheral walls formed with a series of longitudinally extending and circumferentially spaced water cooling passages supplied with cooling water through the roll ends from water supply ducts in the roll drive shafts 41 which are connected to water supply hoses 42 through rotary glands 43. The rolls may typically be about 500 mm diameter and up to 1300 mm long in order to produce 1300 mm wide strip product.

Ladle 17 is of entirely conventional construction and is supported via a yoke 45 on an overhead crane whence it can be brought into position from a hot metal receiving station. The ladle is fitted with a stopper rod 46 actuable by a servo cylinder to allow molten metal to flow from the ladle through an outlet nozzle 47 and refractory shroud 48 into tundish 18.

Tundish 18 is also of conventional construction. It is formed as a wide dish made of a refractory material such as magnesium oxide (MgO). One side of the tundish receives molten metal from the ladle and is provided with the aforesaid overflow 24 and emergency plug 25. The other side of the tundish is provided with a series of longitudinally spaced metal outlet openings 52. The lower part of the tundish carries mounting brackets 53 for mounting the tundish onto the roll carriage frame 31 and provided with apertures to receive indexing pegs 54 on the carriage frame so as to accurately locate the tundish.

Delivery nozzle 19 is formed as an elongate body made of a refractory material such as alumina graphite. Its lower part is tapered so as to converge inwardly and downwardly so that it can project into the nip between casting rolls 16. It is provided with a mounting bracket 60 whereby to support it on the roll carriage frame and its upper part is formed with outwardly projecting side flanges 55 which locate on the mounting bracket.

Nozzle 19 may have a series of horizontally spaced generally vertically extending flow passages to produce a suitably low velocity discharge of metal throughout the width of the rolls and to deliver the molten metal into the nip between the rolls without direct impingement on the roll surfaces at which initial solidification occurs. Alternatively, the nozzle may have a single continuous slot outlet to deliver a low velocity curtain of molten metal directly into the nip between the rolls and/or it may be immersed in the molten metal pool.

The pool is confined at the ends of the rolls by a pair of side closure plates 56 which are held against stepped ends 57 of the rolls when the roll carriage is at the casting station. Side closure plates 56 are made of a strong refractory material, for example boron nitride, and have scalloped side edges 81 to match the curvature of the stepped ends 57 of the rolls. The side plates can be mounted in plate holders 82 which are movable at the casting station by actuation of a pair of hydraulic cylinder units 83 to bring the side plates into engagement with the stepped ends of the casting rolls to form end closures for the molten pool of metal formed on the casting rolls during a casting operation.

During a casting operation the ladle stopper rod 46 is actuated to allow molten metal to pour from the ladle to the tundish through the metal delivery nozzle whence it flows to the casting rolls. The clean head end of the strip product 20 is guided by actuation of an apron table 96 to the jaws of the coiler 21. Apron table 96 hangs from pivot mountings 97 on the main frame and can be swung toward the coiler by actuation of an hydraulic cylinder unit 98 after the clean head end has been formed. Table 96 may operate against an upper strip guide flap 99 actuated by a piston and a cylinder unit 101 and the strip product 20 may be confined between a pair of vertical side rollers 102. After the head end has been guided in to the jaws of the coiler, the coiler is rotated to coil the strip product 20 and the apron table is allowed to swing back to its inoperative position where it simply hangs from the machine frame clear of the product which is taken directly onto the coiler 21. The resulting strip product 20 may be subsequently transferred to coiler 22 to produce a final coil for transport away from the caster.

It has been found in the operation of the above described apparatus that it is possible to consistently produce good austenitic stainless steel strip by careful adjustment of the steel chemistry in combination with the use of rolls having textured surfaces to minimise segregation through initial rapid cooling rates.

In austenitic stainless steel strip casting, solidification mode can play an important part in determining strip surface quality. Primary austenitic solidification mode which occurs when the Cr/Ni ratio is less than about 1.60 is not usually recommended as segregation is enhanced leading to an increase in cracking tendency. It has previously been thought necessary to ensure a Cr/Ni ratio within the range 1.7 to 1.9 in order to minimise cracks due to a reduction in segregation severity and to provide tortuous paths making crack propagation difficult. However our experimental work has shown that continuous strip casting with steel of this composition is very prone to produce strips with "crocodile skin" depressions and the depression severity may be so high as to cause cracking. Steel with Cr/Ni ratio less than 1.55 is most prone to segregation and can thus increase cracking. If solidification occurs on a smooth substrate initial heat transfer rates are low and the solidification structure is coarse resulting in segregation and cracking. However we have determined that this tendency to segregation and cracking can be overcome by ensuring a high initial heat transfer rate and this can most readily be achieved by using a textured substrate, for example by the machining of ridges in the substrate surface.

Initial experimental work was carried out in a metal solidification test rig in which a 40 mm x 40 mm chilled block is plunged into a bath of molten steel at such a speed as to closely simulate the conditions at the casting surfaces of a twin roll caster. Steel solidifies onto the chilled block as it moves through the molten bath to produce a layer of solidified steel on the surface of the block. The thickness of this layer can be measured at points throughout its area to map variations in the solidification rate and therefore the effective rate of heat transfer at the various locations. It is thus possible to produce an overall solidification constant, generally indicated by the symbol K, as well as a map of individual values throughout the solidified strip. It is also possible to examine the micro structure of the strip surface to correlate changes in the solidification micro structure with the changes in the observed heat transfer values.

The nature of the experimental work and the results obtained will now be described.

### EXPERIMENTAL CONDITIONS

Tests were conducted on three copper substrates with different surface characteristics; a smooth and a textured copper surface and a Cr coated (100 µm in thickness), ground surface. Texture was imparted to the copper block by machining longitudinal grooves and ridges with geometry shown schematically in Figure 6. Each of these blocks was instrumented with thermocouples to characterise the heat transfer rates prevailing during solidification. In order to maintain consistent casting conditions throughout the experiments, variables such as melt superheat and block temperature were kept constant within reasonable limits. The melt temperature was aimed at about 1525°C corresponding to a superheat of 75°C. Argon gas introduced into the furnace was quite effective in preventing chemical interaction of the melt with the surrounding atmosphere. The melt chemistry was adjusted to achieve the desired (Cr/Ni)_{eq} ratios, primarily through additions of Cr, Ni, C and N₂. The following expressions were used to determine Cr_{eq} and Ni_{eq}:

Cr_{eq} = Cr + 1.37 Mo + 1.50 Si + 2.0 Nb + 3.0 Ti (1)

Ni_{eq} = Ni + 0.31 Mn + 22.0 C + 14.2 N + Cu (2)

A summary of the test conditions is contained in Table 1. The entire experimental program comprised approximately 45 tests with (Cr/Ni)_{eq} ratios varying between 1.55 and 1.74. Salient features of various tests are summarised in Table 2.

**Table 1**

| Experimental conditions | |
|---|---|
| Substrate surface | Smooth copper Cr plated (ground) copper Textured copper (150µm pitch, 20µm depth) |
| Substrate cleaning procedure | Bristle brush and air blowing |
| Melt temperature | 1525°C |
| Block temperature | 125°C |

**Table 2**

| Details of the various tests | | | | |
|---|---|---|---|---|
| CONDITION | (Cr/Ni)_{eq} | MELT N₂ | GAS ATM | TOTAL DIPS |
| 1 | 1.56-1.71 | 0.047 | Ar | 9 |
| 2 | 1.58-1.71 | 0.037 | Ar | 9 |
| 3 | 1.57-1.61 | <0.062 | N₂ | 7 |
| 4 | 1.59 | 0.062 | Ar | 7 |
| 5 | 1.74 | 0.054-0.059 | Ar Ar + He | 15 |

### RESULTS

### Effect of (Cr/NI)_{eq} ratio on strip surface quality

Visual examination of the samples revealed that (Cr/Ni)_{eq} ratio has a direct influence on the surface quality of the strip obtained with a textured substrate, however, no noticeable effect could be seen with the smooth substrates. Samples cast at varying (Cr/Ni)_{eq} ratio, reveal a gradual progression from a severe crocodile skin type texture to a smooth surface texture with decreasing (Cr/Ni)_{eq} ratio. The effect of (Cr/Ni)_{eq} ratio on crocodile skin severity, shown in Figure 9, suggests that substantial improvements in strip surface quality can be achieved by keeping the (Cr/Ni)_{eq} ratio less than 1.60.

### Effect of (Cr/Ni)_{eq} ratio on heat transfer during solidification

### i) Textured substrate

Heat transfer rates from the strip surface to the substrate were determined from the measured substrate temperatures. Figure 7 shows the influence of melt (Cr/Ni)_{eq} ratio on heat fluxes for a textured substrate. It can be seen that the profiles are characterised by an early peak in the heat flux followed by rapid reduction of this peak and with increasing time, heat flux approaches a constant value. Higher heat transfer rates (about 30 MW/m²) encountered in the early stages of solidification can be attributed to the intimate contact.

The experimental program determined that the (Cr/Ni)_{eq} ratio found to producing the best surface texture (on a textured substrate) is less than 1.60.

### ii) Smooth substrate

Figure 8 reveals the influence of (Cr/Ni)_{eq} ratio on heat transfer for a smooth substrate. It can be seen that the heat fluxes are relatively constant throughout solidification and most importantly, the magnitudes of the peak fluxes are much lower than those measured for a textured substrate (Figure 7). This finding is in agreement with the observed solidification structure which is coarse at the surface. Although there are some variations in heat flux at different (Cr/Ni)_{eq} ratios, there are no definite trends. However, with increasing time the heat fluxes approach similar values irrespective of (Cr/Ni)_{eq}. This apparent lack of dependence of heat transfer on (Cr/Ni)_{eq} ratio with a smooth substrate is in agreement with the observations of strip surface texture which was not influenced by (Cr/Ni)_{eq}.

The experimental program demonstrated that the normal operating window for (Cr/Ni)_{eq} ratios of 1.7-1.9 is not the optimum in terms of strip surface texture. Using a (Cr/Ni)_{eq} ratio less than 1.60 produces better surface quality.

## Claims

1. A method of continuously casting metal strip of the kind in which a casting pool of molten metal is formed in contact with a moving casting surface such that metal solidifies from the pool onto the moving casting surface, wherein the metal is an austenitic stainless steel containing chromium and nickel in a ratio (Cr/Ni)eq of less than 1.60, the casting surface is textured so as to have an Arithmetical Mean Roughness Value (Rₐ) in the range of 2.5 to 15 microns and heat is transferred from said austenitic stainless steel solidifying onto said textured surface at an initial heat transfer rate of more than 15 MW/m² during the initial 20ms to enable the solidification of said steel on the casting surface without deleterious segregation and surface cracking.

2. A method as claimed in claim 1, wherein the casting surface has a texture of regular grooves and ridges.

3. A method as claimed in claim 2, wherein the texture depth is in the range of 10 microns to 60 microns and the groove pitch is in the range 100 microns to 200 microns.

4. A method as claimed in claim 1, wherein the casting surface has a texture of regularly spaced discrete projections at a pitch spacing in the range 100 to 200 microns and a texture depth in the range 10 to 60 microns.

5. A method as claimed in any one of the preceding claims, wherein the chromium to nickel ratio is no greater than 1.55.

6. A method as claimed in any one of the preceding claims, wherein the carbon, chromium and nickel contents of the steel are in the following ranges:
| | |
|---|---|
| Carbon - | 0.04-0.06% by weight |
| Chromium - | 17.5-19.5% by weight |
| Nickel- | 8.0-10.0% by weight |

7. A method of continuously casting metal strip of the kind in which molten metal is introduced into the nip between a pair of casting rolls via a metal delivery nozzle disposed above the nip to create a casting pool of molten metal supported on casting surfaces of the rolls immediately above the nip, wherein the metal is an austenitic stainless steel containing chromium and nickel in a ratio (Cr/Ni) eq of less than 1.60, the casting surfaces are textured so as to have an Arithmetical Mean Roughness Value (Rₐ) in the range 2.5 to 15 microns and heat is transferred from said austenitic stainless steel solidifying onto said textured casting surfaces of the rolls at an initial heat transfer of more than 15 MW/m² during the initial 20ms to enable the solidification of said steel on the casting surfaces without deleterious segregation and cracking.

8. A method as claimed in claim 7, wherein the casting surfaces of the rolls have a texture of regular circumferential grooves with a texture depth in the range 10 microns to 60 microns and a groove pitch in the range 100 microns to 200 microns.

9. A method as claimed in claim 7, wherein the rolls have a texture of regularly spaced discrete projections at a pitch spacing in the range 100 to 200 microns and a depth in the range 10 to 60 microns.

10. A method as claimed in any of claims 7 to 9, wherein the chromium to nickel ratio is no greater than 1.55.

11. A method as claimed in any one of claims 7 to 10, wherein the carbon, chromium and nickel of the steel are in the following ranges:
| | |
|---|---|
| Carbon - | 0.04-0.06% by weight |
| Chromium - | 17.5-19.5% by weight |
| Nickel - | 8.0-10.0% by weight |

## Patentansprüche

1. Verfahren zum Stranggießen von Metallband der Art, bei der ein Gießbad aus geschmolzenem Metall in Kontakt mit einer sich bewegenden Gießoberfläche ausgebildet wird, so daß Metall aus dem Bad auf der sich bewegenden Gießoberfläche erstarrt, wobei das Metall ein austenitischer nichtrostender Stahl ist, der Chrom und Nickel in einem Verhältnis (Cr/Ni)_{eq} von weniger als 1,60 enthält und die Gießoberfläche so texturiert ist, dass sie einen arithmetischen Rauhigkeitsmittelwert (Rₐ) im Bereich von 2,5 bis 15 µm hat, und Wärme von dem austhenitischen nichtrostenden Stahl, der auf den texturierten Gießoberflächen der Walzen erstarrt, mit einer anfänglichen Wärmeübergangsrate von mehr als 15 MW/cm² in den ersten 20 ms übertragen wird, um die Erstarrung des Stahls auf den Gießoberflächen ohne schädliche Seigerung und Oberflächenrißbildung zu ermöglichen.

2. Verfahren nach Anspruch 1, wobei die Gießoberfläche eine Textur aus regelmäßigen Rillen und Rippen hat.

3. Verfahren nach Anspruch 2, wobei die Texturtiefe im Bereich von 10 µm bis 60 µm liegt und der Rillenabstand im Bereich von 100 µm bis 200 µm liegt.

4. Verfahren nach Anspruch 1, wobei die Gießoberfläche eine Textur aus regelmäßig beabstandeten getrennten Vorsprüngen in einem Abstand im Bereich von 100 bis 200 µm und eine Texturtiefe im Bereich von 10 bis 60 µm hat.

5. Verfahren nach einem der vorhergehenden Ansprüche, wobei das Verhältnis zwischen Chrom und Nickel nicht größer als 1,55 ist.

6. Verfahren nach einem der vorhergehenden Ansprüche, wobei der Kohlenstoff-, Chrom- und Nickelgehalt des Stahls in den folgenden Bereichen liegen:
| | |
|---|---|
| Kohlenstoff - | 0,04 bis 0,06 Gew.-% |
| Chrom - | 17,5 bis 19,5 Gew.-% |
| Nickel - | 8,0 bis 10,0 Gew.-%. |

7. Verfahren zum Stranggießen von Metallband der Art, bei der geschmolzenes Metall in den Spalt zwischen einem Paar Gießwalzen durch eine Metallaustrittsdüse eingebracht wird, die über dem Spalt angeordnet ist, um ein Gießbad aus geschmolzenem Metall zu erzeugen, das auf Gießoberflächen der Walzen unmittelbar über dem Spalt gehalten wird, wobei das Metall ein austhenitischer nichtrostender Stahl ist, der Chrom und Nickel in einem Verhältnis (Cr/Ni) von weniger als 1,60 enthält, die Gießoberflächen so texturiert sind, dass sie einen arithmetischen Rauhigkeitsmittelwert (Rₐ) in dem Bereich von 2,5 bis 15 µm haben, und Wärme von dem austhenitischen nichtrostenden Stahl, der auf den texturierten Gießoberflächen der Walzen erstarrt, mit einer anfänglichen Wärmeübergangsrate von mehr als 15 MW/cm² in den ersten 20 ms übertragen wird, um die Erstarrung des Stahls auf den Gießoberflächen ohne schädliche Seigerung und Oberflächenrißbildung zu ermöglichen.

8. Verfahren nach Anspruch 7, wobei die Gießoberflächen der Walzen eine Textur aus regelmäßigen Umfangsrillen mit einer Texturtiefe im Bereich von 10 µm bis 60 µm und einem Rillenabstand im Bereich von 100 µm bis 200 µm haben.

9. Verfahren nach Anspruch 7, wobei die Walzen eine Textur von regelmäßig beabstandeten getrennten Vorsprüngen in einem Abstand im Bereich von 100 bis 200 µm und einer Tiefe im Bereich von 10 bis 60 µm haben.

10. Verfahren nach einem der Ansprüche 7 bis 9, wobei das Verhältnis zwischen Chrom und Nickel nicht größer als 1,55 ist.

11. Verfahren nach einem der Ansprüche 7 bis 10, wobei der Kohlenstoff-, Chrom- und Nickelgehalt des Stahls in den folgenden Bereichen liegt:
| | |
|---|---|
| Kohlenstoff - | 0,04 bis 0,06 Gew.-% |
| Chrom - | 17,5 bis 19,5 Gew.-% |
| Nickel - | 8,0 bis 10,0 Gew.-%. |
Wärme von dem austhenitischen nichtrostenden Stahl, der auf den texturierten Gießoberflächen der Walzen erstarrt, mit einer anfänglichen Wärmeübergangsrate von mehr als 15 MW/cm² in den ersten 20 ms übertragen wird, um die Erstarrung des Stahls auf den Gießoberflächen ohne schädliche Seigerung und Oberflächenrißbildung zu ermöglichen.

## Revendications

1. Procédé de coulée continue d'une bande de métal du type dans lequel une masse de coulée de métal fondu est formée au contact d'une surface de coulée mobile de telle sorte que du métal se solidifie à partir de la masse sur la surface de coulée mobile, dans lequel le métal est un acier inoxydable austénitique contenant du chrome et du nickel selon un rapport (Cr/Ni)_{éq} inférieur à 1,60, la surface de coulée a une texture telle que la valeur arithmétique moyenne de rugosité (Ra) est comprise dans la gamme de 2,5 à 15 µm et que la chaleur est transférée à partir dudit acier inoxydable austénitique qui se solidifie sur la surface de coulée texturée à une vitesse initiale de transfert de chaleur supérieure à 15 MW/m² au cours des 20 ms initiales pour permettre la solidification dudit acier sur la surface de coulées sans ségrégation ni fissuration de surface nuisible.

2. Procédé suivant la revendication 1, dans lequel la surface de coulée présente une texture de rainures et d'arêtes régulières.

3. Procédé suivant la revendication 2 dans lequel la profondeur de la texture est comprise dans la gamme de 10 µm à 60 µm et le pas des rainures est compris dans la gamme de 100 µm à 200 µm.

4. Procédé suivant la revendication 1, dans lequel la surface de coulée a une texture de protubérances discrètes régulièrement espacées avec un pas compris dans la gamme de 100 à 200 µm et une profondeur de texture comprise dans la gamme de 10 à 60 µm.

5. Procédé suivant l'une quelconque des revendications précédentes, dans lequel le rapport du chrome au nickel ne dépasse pas 1,55.

6. Procédé suivant l'une quelconque des revendications précédentes, dans lequel les teneurs en carbone, chrome et nickel de l'acier sont comprises dans les gammes suivantes :
| | |
|---|---|
| Carbone | 0,04 à 0,06 % en poids |
| Chrome | 17,5 à 19,5 % en poids |
| Nickel | 8,0 à 10,0 % en poids |

7. Procédé de coulée continue d'une bande de métal du type dans lequel du métal fondu est introduit dans la pince formée entre deux rouleaux de coulée par l'intermédiaire d'une buse de distribution de métal située au-dessus de la pince pour créer une masse de coulée de métal fondu supportée sur des surfaces de coulée des rouleaux immédiatement au-dessus de la pince, dans lequel le métal est un acier inoxydable austénitique contenant du chrome et du nickel selon un rapport (Cr/Ni)eq inférieur à 1,60, les surfaces de coulée ont une texture telle qu'elles ont une Valeur arithmétique moyenne de rugosite (Ra) comprise dans la gamme de 2,5 à 15 microns et la chaleur est transférée à partir dudit acier inoxydable austénitique qui se solidifie sur les surfaces de coulée texturées des rouleaux à une vitesse initiale de transfert de chaleur supérieure à 15 MW/m² au cours des 20 ms initiales pour permettre la solidification dudit acier sur les surfaces de coulées sans ségrégation ni fissuration.

8. Procédé suivant la revendication 7, dans lequel les surfaces de coulée des rouleaux présentent une texture de rainures circonférentielles régulières avec une profondeur de texture comprise dans la gamme de 10 µm à 60 µm et un pas des rainures compris dans la gamme de 100 µm à 200 µm.

9. Procédé suivant la revendication 7, dans lequel les rouleaux ont une texture de protubérances discrètes régulièrement espacées avec un pas d'espacement compris dans la gamme de 100 µm à 200 µm et une profondeur de texture comprise dans la gamme de 10 µm à 60 µm.

10. Procédé suivant l'une quelconque des revendications 7 à 9, dans lequel le rapport du chrome au nickel ne dépasse pas 1,55.

11. Procédé suivant l'une quelconque des revendications 7 à 10, dans lequel les teneurs en carbone, chrome et nickel de l'acier sont comprises dans les gammes suivantes :
| | |
|---|---|
| Carbone | 0,04 à 0,06% en poids |
| Chrome | 17,5 à 19,5% en poids |
| Nickel | 8,0 à 10,0% en poids |
